

1,241,618.

E. GATHMANN,  
INGOT AND INGOT MOLD.  
APPLICATION FILED NOV. 23, 1912.

Patented Oct. 2, 1917.

2 SHEETS—SHEET 1.



Fig. 2.



Fig. 4.



Fig. 1.

Fig. 3.



Fig. 5.



Inventor

Witnesses

Alfred Murray,  
C. B. Franzoni.



Emil Gathmann

By his Attorneys  
Baldwin Wright

1,241,618.

E. GATHMANN,  
INGOT AND INGOT MOLD,  
APPLICATION FILED NOV. 23, 1912.

Patented Oct. 2, 1917.  
2 SHEETS—SHEET 2.

Fig. 7.



Fig. 8.



Fig. 9.



Witnesses

H. L. Murray  
E. B. Franzoni.

Inventor

a<sup>2</sup> Emil Gathmann  
by his Attorneys  
Burdette & Wright

# UNITED STATES PATENT OFFICE.

EMIL GATHMANN, OF BALTIMORE, MARYLAND.

## INGOT AND INGOT-MOLD.

1,241,618.

Specification of Letters Patent.

Patented Oct. 2, 1917.

Application filed November 23, 1912. Serial No. 733,062.

*To all whom it may concern:*

Be it known that I, EMIL GATHMANN, a citizen of the United States, residing in Baltimore city, State of Maryland, have 5 invented certain new and useful Improvements in Ingots and Ingot-Molds, of which the following is a specification.

This invention relates to the manufacture of ingots and particularly to the manufacture of ingots of crucible steel. It has been found by numerous experiments that when 10 the mold cavity is larger at its upper than at its lower end and gradually tapers toward the lower end, where the cross section 15 is smaller, the lower portion of the ingot freezes or solidifies more quickly as less heat units are contained therein than in the larger portion of the mold. This tapering of the mold cavity should be progressive 20 but uniform, *i. e.*, there should not be any sudden change in taper as that would cause the ingot to hang at some point of the mold. With the ordinary tapered ingot for crucible 25 steel practice, it has been found that difficulty has been encountered in stacking or piling the ingots for storage on account of their varying dimensions from end to end, and it has also been found difficult to work such ingots under the steam hammer or hydraulic press. Notwithstanding these 30 troubles, such ingots have been and are now very extensively used.

By my improvements I produce tapered ingots of such form that they may be readily and uniformly stacked and worked under the hammer or press and which are practically free from pipes or blow holes.

By my invention I obtain uniform cross section of the ingot in certain longitudinal 40 planes but a decreased cross section with consequent change of dimensions in another longitudinal cross section. This I do by leaving some of the sides of the ingot straight, flat and parallel, while others are 45 tapered.

My improvements are illustrated in the accompanying drawings, in which,

Figure 1 shows a vertical central section through a mold for forming an ingot embodying my improvements.

Fig. 2 shows a top plan view thereof.

Fig. 3 shows a side elevation of one section of the mold illustrated in Fig. 1.

Fig. 4 shows a top plan view of the form 55 of mold shown in Figs. 1 and 3, both sections of the mold being illustrated,

Fig. 5 shows a transverse section on the line 5—5 of Fig. 1.

Fig. 6 shows a bottom plan view of the mold shown in Fig. 1.

Fig. 7 shows a vertical central section through a non-sectional or solid mold for forming an ingot embodying my improvements.

Fig. 8 is a perspective view with parts 65 broken away of an ingot embodying my invention.

Fig. 9 illustrates how the ingots may be stacked or piled.

The mold B may be made in sections, as 70 shown in Figs. 1 to 6 inclusive, or it may be solid, as indicated in Fig. 7. In either case the walls of the mold are preferably made thicker in the lower portion thereof and relatively thin at the upper or neck 75 portion, as by such construction the lower portion of the mold absorbs heat rapidly from the ingot, while the thin upper portion or neck is less absorbent. In this way the pipe which ordinarily forms in the process of manufacture is forced to the top where it disappears or dwells near the upper end of the ingot, leaving a relatively small crop end. When the mold is made in sections as 80 shown in Figs. 1 to 6, suitable devices are 85 employed for securing the sections together as is usual in this art.

The shape of the preferred form of mold cavity can be readily understood by reference to the illustration of the ingot, A 90 shown in Fig. 8. The cavity, of course, must correspond substantially in shape with the ingot. It will be observed that the ingot has a substantially square or rectangular upper end  $a$  and it has four sides  $a'$  which are substantially straight, parallel and flat. Between these four sides  $a'$  there are four other sides  $a''$  which taper from the upper portion of the ingot downwardly, gradually increasing in width toward the lower 100 end of the ingot. In this way the ingot has flat sides which enable it to be placed on top of another similar ingot parallel with it. In this way also any desired number of ingots may be piled or stacked without danger of toppling over and with great compactness.

Referring now to the mold cavity, it will be observed that it has some of its walls substantially straight, flat and parallel and others tapered from the top of the mold toward the bottom thereof. The straight, flat 110

and parallel sides of the mold cavity are indicated at  $b$  and the tapered sides at  $b'$ . The bottom of the mold cavity is preferably slightly rounded at  $b^s$  to produce the rounded end  $\alpha^s$  at the bottom of the ingot.

By reference to Fig. 6, for instance, it will be observed that the mold cavity, and consequently the ingot is approximately square at both top and bottom in cross section, the smaller square being inscribed within the top or larger square. By this construction I obtain the advantages of a big end up or tapered ingot without the disadvantages or troubles usually encountered in stacking and in hammering or cobbing down of the ingot. Where the mold is solid, as indicated in Fig. 7, a very slight taper should be given to the walls and cavity in order that the ingot may be readily withdrawn from the mold after it has solidified.

In the preferred construction the ingot has approximately parallel walls at four of its sides and tapering walls intervening between these four side walls and said ingot has a cross section at its top portion approximately 1.5 times as large as the cross section of the lower end of the ingot. Four of the side walls are practically parallel from the larger to the smaller cross section.

I claim as my invention:

1. An ingot having two of its opposite sides approximately straight and equidistant from the vertical central axis of the

ingot at its upper and lower portions and 35 two intervening sides inclined and converging from the top toward the ingot bottom.

2. A metallic mold in which the mold cavity has some of its sides approximately 40 straight and parallel while others are relatively tapered or inclined from the upper end of the mold downwardly toward the bottom thereof.

3. A metallic mold in which the mold cavity has some of its sides approximately 45 straight and parallel, while others are relatively tapered or inclined from the upper end of the mold downwardly toward the bottom thereof, said mold cavity being of greater cross section at top than at bottom 50 and the walls of said mold being made to absorb heat more rapidly at its lower portion than at its upper portion.

4. A metallic mold, in which the mold cavity has some of its sides approximately 55 straight and parallel while others are relatively tapered or inclined from the upper end of the mold downwardly toward the bottom thereof, the walls on diametrically opposite sides of the mold cavity at the 60 lower portion of the mold being thicker than the remaining or intervening walls.

In testimony whereof, I have hereunto subscribed my name.

EMIL GATHMANN.

Witnesses:

ALEX. C. GROOME,  
JOSHUA S. HULL.